

# United States Patent

Amano et al.

[15] 3,650,752  
[45] Mar. 21, 1972

[54] **WHITENED PHOTOGRAPHIC PRINTING PAPER**

- [72] Inventors: **Hiroyuki Amano; Nobuo Tsuji; Takushi Miyazako; Kazuo Shirasu; Yosinori Tutiya**, all of Kanagawa, Japan
- [73] Assignee: **Fuji Photo Film Co.**, Ashigara-Kamigun, Kanagawa, Japan
- [22] Filed: **May 12, 1970**
- [21] Appl. No.: **36,525**

[30] **Foreign Application Priority Data**

- May 12, 1969 Japan.....44/36404
- [52] U.S. Cl.....96/82, 117/33.5 T, 96/85
- [51] Int. Cl.....G03c 1/92
- [58] Field of Search.....96/82; 117/33.5 T

[56]

**References Cited**

**UNITED STATES PATENTS**

- |           |        |                    |       |
|-----------|--------|--------------------|-------|
| 3,047,390 | 7/1962 | Koerber et al..... | 96/82 |
| 3,181,948 | 5/1965 | Koerber et al..... | 96/82 |
| 3,269,840 | 8/1966 | Pattyn et al.....  | 96/82 |

*Primary Examiner*—Ronald H. Smith

*Attorney*—Sughrue, Rothwell, Mion, Zinn and Macpeak

[57]

**ABSTRACT**

A photographic printing paper comprising a support having thereon a light-sensitive silver halide emulsion layer containing a water-soluble fluorescent brightening agent and a partially urethanated polyvinyl alcohol having the following recurring structure:



wherein  $x+y$  is a number from 100 to 5,000 and  $y/(x+y)$  is a number from 0.05 to 0.25.

**14 Claims, 1 Drawing Figure**

Patented March 21, 1972

3,650,752



INVENTORS

HIROYUKI AMANO  
NOBUO TSUJI  
TAKUSHI MIYAZAKO  
KAZUO SHIRASU  
YOSINORI TUTIYA

BY

*Sugars, Estwell, Lewin,  
Zinn & Macpeak*  
ATTORNEYS

## WHITENED PHOTOGRAPHIC PRINTING PAPER

## BACKGROUND OF THE INVENTION

## 1. Field of the Invention

This invention relates to photographic printing paper having an improved whiteness and, more particularly, photographic printing paper of improved whiteness achieved by incorporating a fluorescent brightening agent and a partially urethanated polyvinyl alcohol in the photographic printing paper to increase the fluorescent brightening action.

## 2. Description of the Prior Art

It is known as a means for whitening a photographic printing paper to incorporate in the photographic emulsion layer or a subsidiary layer such as a protective layer, an intermediate layer, an undercoating, or a baryta layer, a fluorescent brightening agent emitting from violet to blue fluorescence when irradiated by ultraviolet light.

However, since fluorescent brightening agents have a dyeing affinity directly to fibers, etc., they show less of a dyeing affinity to the binders for the photographic emulsion layers or subsidiary layers, such as gelatin, and thus there is the disadvantage that the greater part of the fluorescent brightening agent is diffused in a conventional whitened photographic printing paper during photographic processing and washing, whereby the brightening effect is lost.

Therefore, in order to solve this problem, various investigations have been undertaken for increasing the brightening effect by using combinations of fluorescent brightening agents and various kinds of high molecular weight compounds. For instance, since a fluorescent brightening agent has a low dyeing affinity to gelatin, there have been provided various methods of dyeing gelatin with a fluorescent brightening agent including preliminarily dispersing in the gelatin polyvinyl pyrrolidone or poly-N-vinyl-5-methyl-2-oxazolidinone (U.S. Pat. No. 3,269,840), which has a good dyeing affinity to the fluorescent brightening agent. However, even if such high molecular weight compounds are used, the dyeing of the fluorescent brightening agent is insufficient and the agent is also diffused during photographic processing and washing. Further, such high molecular weight compounds show a higher brightening effect as the molecular weight thereof is higher but if the degree of polymerization is increased, the compatibility thereof with gelatin as a binder is reduced and phase separation results, and therefore the use of high molecular weight compounds having a high degree of polymerization is accompanied by such disadvantages that significant trouble occurs during the coating step in the preparation of photographic light-sensitive materials and even if the coating procedure can be practiced, the resulting surface is matted in the case of producing glossy photographic printing papers.

Also, there has also been proposed a method wherein a copolymer of N-vinylpyrrolidone and vinyl acetate, styrene, acrylate or methacrylate is used together with a fluorescent brightening agent (Japanese Pat. publication No. 22882/68). However, although the copolymer may withstand photographic processing and washing for a long time as compared with polyvinyl pyrrolidone having the same molecular weight as the copolymer, the compatibility of the copolymer with gelatin is lower than that of polyvinyl pyrrolidone with gelatin and thus the disadvantage of phase separation is more likely to occur and the surface of glossy photographic printing paper becomes more matted.

Still another proposed solution has been the use of a combination of an ethyl acrylate-vinyl isobutyl ether-styrene-acrylic acid copolymer and a cumarinic oil-soluble type fluorescent brightening agent (Belgian Pat. No. 646,150). However, this combination has the disadvantage that while the copolymer may be sufficient from the point of view of preventing diffusion, the copolymer has a significantly less fluorescent brightening effect than polyvinyl pyrrolidone.

Therefore, an object of the present invention is to provide a photographic printing paper having improved whiteness.

Another object of the present invention is to provide a photographic printing paper containing a fluorescent brightening agent. A still further object of the present invention is to provide a photographic printing paper having an improved whiteness even after being subjected to various photographic processings. A still further object of the present invention is to provide a photographic printing paper having good whiteness and a good surface property.

## SUMMARY OF THE INVENTION

The above objects of the present invention can be achieved by incorporating in an emulsion layer or a subsidiary layer of a photographic printing paper a water-soluble fluorescent brightening agent and a partially urethanated polyvinyl alcohol having the following recurring structure:



wherein  $x+y=100$  to 5,000 and  $y/(x+y)=0.05$  to 0.25

## BRIEF DESCRIPTION OF THE DRAWING

The figure represents the fluorescent intensity of printing papers produced according to the present invention in comparison to other printing papers.

## DETAILED DESCRIPTION OF THE PREFERRED EMBODIMENTS

The term "photographic printing paper" as used in the present specification, includes not only black and white photographic printing paper and color photographic printing paper but also light-insensitive positive material for diffusion transfer photographic processes. The term "subsidiary layer" includes light-insensitive layers for photographic printing papers, such as a protective layer, an intermediate layer, and undercoating, a baryta layer and an image receiving layer for diffusion transfer photographic paper.

The desirable feature obtained by using the combination of a fluorescent brightening agent and a partially urethanated polyvinyl alcohol according to the present invention are shown below. 1. A remarkable brightening effect is obtained as compared with the case of adding the fluorescent brightening agent alone.

2. The partially urethanated polyvinyl alcohol of this invention shows a larger fluorescent brightening effect as the degree of polymerization thereof becomes higher as is the case with the known high molecular weight compounds such as polyvinyl pyrrolidone, poly-N-vinyl-5-methyl-2-oxazolidinone, N-vinyl pyrrolidone-vinyl acetate copolymer, N-vinyl pyrrolidone-acrylate copolymer, N-vinyl pyrrolidone-styrene copolymer, and N-vinyl pyrrolidone-methacrylate copolymer. However, as the compatibility thereof with gelatin is good when the degree of polymerization thereof is high, no trouble during the coating step in the production of photographic light-sensitive materials nor matting of the surface of glossy photographic printing papers occurs.

3. Since the partially urethanated polyvinyl alcohol of this invention has a better dyeing affinity to the fluorescent brightening agent than the above-mentioned known compounds as well as having a good dyeing affinity to gelatin, a larger fluorescent brightening effect can be obtained not only when the molecular weight thereof is the same as that of the above-mentioned known compounds but even when it is lower than the molecular weight of the latter compounds even after the photographic printing paper is subjected to photographic processing and washing.

4. It is known that polyvinyl pyrrolidone is an effective medium for the polymer latex used as a baryta composition for photographic printing paper (Dutch Pat. publication No. 6,705,734) but the partially urethanated polyvinyl alcohol of this invention is also as effective as polyvinyl pyrrolidone.

It is desirable that the partially urethanated polyvinyl alcohol of this invention have a high urethanated ratio, but too high a urethanation ratio is undesirable since, as a result, the water-solubility thereof is reduced. Therefore, the urethanation ratio of the partially urethanated polyvinyl alcohol may vary from 5 to 25 percent and preferably from 7 to 20 percent. Also, the degree of polymerization may vary from 100 to 5,000, and preferably from 1,500 to 3,000, referring to the expression  $x+y$  described above.

The partially urethanated polyvinyl alcohol may be readily prepared by the reaction of polyvinyl alcohol and urea. For instance, the compound prepared by heating polyvinyl alcohol and urea in formamide or dimethyl formamide to 100° C. is shown in Pat. publication No. Sho 37-1,3886. Also, it may be prepared by the method disclosed in Pat. publication No. Sho 37-692 and Pat. publication No. Sho 40-18,863. However, the method of preparing the partially urethanated polyvinyl al-

Benzidine type fluorescent brightening agent:



wherein R and R' each represents -h, -CH3 or -OCH3, or



15 wherein R and R' each represents -H, -CH3 or -OCH3.

Triazole type fluorescent brightening agent:



cohol of this invention is not limited and any suitable method can be employed.

Typical examples of the partially urethanated polyvinyl alcohol according to the present invention are shown below:

Compound 1. The 14 percent-urethanated product of polyvinyl alcohol having a polymerization degree of 2,400.

Compound 2. The 15 percent-urethanated product of polyvinyl alcohol having a polymerization degree of 1,700.

Compound 3. The 13 percent-urethanated product of polyvinyl alcohol having a polymerization degree of 2,400.

Compound 4. The 7 percent-urethanated product of polyvinyl alcohol having a polymerization degree of 2,400.

The amount added of the partially urethanated polyvinyl alcohol of this invention is influenced by the nature of the layer to which it is added but generally the amount may vary from 1 to 30 percent by weight, based on the weight of the binder of the layer, and preferably, from 5 to 25 percent by weight.

Any suitable water-soluble fluorescent brightening agent having a property of emitting from violet to blue fluorescence by absorbing ultraviolet rays may be used in this invention. Diaminostilbene type, benzidine type, triazole type, imidazole type, and imidazolon type water-soluble fluorescent brightening agents having direct dyeing affinity are known and these known fluorescent brightening agents can be preferably used in accordance with the present invention. Practical examples of these fluorescent brightening agents are shown below.

Diaminostilbene type fluorescent brightening agent:



wherein X, X', Y and Y' each represents -NHC6H5, -NHC6H4SO3Na, -OH, -NH2, -NHCH2CH2SO3Na, -OCH2CH2OH, or -OCH3.



These fluorescent brightening agents are sold under the trade names: "Blankophor" (Bayer A. G., Germany), "Leucophor" (J. R. Geigy A. G., Switzerland), "Tinopal" (Sandoz A. G., Switzerland), "Uvitex" (CIBA A. G., Switzerland), "Kayaphor" (Nippon Kayaku K. K.), "Whitex" (Sumitomo Kagaku Kogyo K. K.), and "YL" (Honshu Kagaku K. K.). For example, "Blankophor B" and "Leucophor B" are fluorescent brightening agents represented by formula (1) above and "Whitex R extra conc" is represented by formula (2) above.

Furthermore, the high molecular weight fluorescent brightening agents previously discovered by the same inventors may also be employed according to the present invention, i.e., the high molecular weight compounds having the repeating units represented by the following general formula (I) or (II)



wherein  $R_1$  and  $R_2$  each represents a hydrogen atom, an alkyl group having one to eight carbon atoms, an aryl group having six to 12 carbon atoms, a hydroxyalkyl group having two to four carbon atoms, substituted derivatives thereof, a sulfoalkyl group having one to four carbon atoms, or an alkali metal or ammonium salt thereof;  $R_1$  represents a halogen atom.



$R$  and  $R'$  each represents a hydrogen atom, an alkyl group having one to 12 carbon atoms, a hydroxyalkyl group having one to 12 carbon atoms, a sulfoalkyl group or an alkali metal or ammonium salt thereof, an aralkyl group, an aryl group having six to 18 carbon atoms, a hydroxyl-, carboxyl- or sulfonic acid-substituted derivative thereof, or an alkali metal or ammonium salt thereof, a cycloalkyl group having six to 10 carbon atoms or a substituted cycloalkyl group;  $A$  represents an alkylene group having four to five carbon atoms or an alkylene group containing a heterocyclic atom or a heterocyclic atomic group;  $Y$  represents an alkylene group having two to 10 carbon atoms or a substituted alkylene group, or an arylene group having six to 18 carbon atoms or a substituted arylene group;  $Z$  represents a divalent heterocyclic atom or a heterocyclic atomic group; and  $m$  is  $O$  or  $1$ .

As the binder for forming an emulsion layer or a subsidiary layer of a photographic printing paper in this invention, gelatin is most generally used but synthetic high molecular weight compounds such as polyvinyl alcohol and polyvinyl acetal may be effectively used.

The fluorescent brightening effect achieved by the use of the fluorescent brightening agent and the partially urethanated polyvinyl alcohol according to this invention, and also, the effect of preventing the fluorescent brightening agent from being diffused by photographic processing and washing according to the present invention are shown experimentally by the following examples, although the invention is intended to be limited to the same.

#### EXAMPLE 1

0.5 g. of "Leucophor B" (trade name) as a fluorescent brightening agent was added to 1 kg. of a gelatino silver halide emulsion containing 50 g. of gelatin and 20 g. of silver chlorobromide having 30 mol percent silver bromide and after further adding additives such as a hardening agent and a wetting agent, the emulsion was coated on a baryta-coated

paper at the rate of 150 g./m.<sup>2</sup> to give Sample A. Further, 10 g. of Compound 1, 10 g. of Compound 2, and 10 g. of Compound 4 were added to the emulsions as prepared above to give Samples B, C and D, respectively. For comparison, 10 g. of polyvinyl pyrrolidone having a degree of polymerization of 2,400 was added to the same emulsion as above instead of the above-described compounds to give Comparison Sample E. These printing papers thus prepared were processed in a developer having the following composition and in a fixing solution having the following composition:

| Developer                            |          |
|--------------------------------------|----------|
| Metal (trade name)                   | 1.0 g.   |
| Sodium sulfite                       | 15.0 g.  |
| Hydroquinone                         | 4.0 g.   |
| Sodium carbonate (1H <sub>2</sub> O) | 27.0 g.  |
| Potassium bromide                    | 1.3 g.   |
| Water to make                        | 1 liter  |
| Fixing Solution                      |          |
| Sodium thiosulfate                   | 240.0 g. |
| Sodium sulfite                       | 15.0 g.  |
| Glacial acetic acid                  | 13.3 g.  |
| Borax                                | 7.5 g.   |
| Potassium alum                       | 15.0 g.  |
| Water to make                        | 1 liter  |

After washing the printing papers thus processed with running water at 15°C., they are dried through a ferotype.

The intensity of fluorescence of the printing papers thus processed was measured, the results of which are shown in the accompanying drawing, wherein the relationship between washing time (by hour) and the relative fluorescence intensity is shown. Measurements of fluorescent intensity were conducted at 1, 5, 12 and 24 hours. The relative fluorescent intensity is shown by a relative value to the whiteness of the surface of printing paper itself which is assumed to be 25. In the figure, Curve A corresponds to Sample A; Curve B, Sample B; Curve C, Sample C; Curve D, Sample D; and Curve E, Sample E, respectively.

As is clear from the Figure, Samples B-D of the present invention had a higher fluorescence intensity than Control Sample A and Comparison E. Also, it was confirmed that the intensity of fluorescence was increased as the degree of polymerization of the water-soluble high molecular weight material increased and also as the urethanation ratio increased. Furthermore, the surface properties of the printing papers B-D of this invention were not reduced.

Almost the same results were obtained when Compound 1, Compound 2 or Compound 4 of this invention was used together with "Blankophor BUP" (trade name), "Whitex BF" (trade name), "Kayaphor S" (trade name), "Tinopal GS" (trade name),

Compound 5



or Compound 6



## EXAMPLE 2

A blue-sensitive silver iodobromide emulsion containing a yellow coupler, 3, 5-dicarboxy-4-(stearoylamidobenzyl)acetanilide was coated on a baryta-coated paper. The coupler was added to the silver halide emulsion as an alkaline aqueous solution thereof. Then, a green-sensitive silver chlorobromide emulsion containing a magenta coupler, 1-(3-sulfo-4-phenoxy)-3-stearoyl-5-pyrazolone and, further a red-sensitive silver chlorobromide emulsion containing a cyan coupler, N-n-octadecyl-1-hydroxy-4-sulfo-2-naphthamide were coated thereon and finally a protective layer was formed on the red-sensitive layer.

The protective layer was formed by adding 100 ml. of a 1 percent aqueous solution of a known fluorescent brightening agent as shown in Example 1 or 100 ml. of 1 percent aqueous solution of a high molecular weight fluorescent brightening agent (Compound 7) having the following repeating unit



to 1 kg. of a 4 percent aqueous gelatin solution followed by coating and drying, or further adding, together with the fluorescent brightening agent, 200 ml. of a 4 percent aqueous solution of high molecular weight compounds 1, 2, or 3 of this invention and 200 ml. of a 4 percent aqueous solution of polyvinyl pyrrolidone followed by coating and drying.

The color photographic printing papers thus produced were developed in a developer containing a color developing agent, N-ethyl-N-β-hydroxyethyl-p-phenylenediamine and after subjecting them to stop-fixing, washing, bleach-fixing, washing, hardening, washing, and drying, the intensity of fluorescence was measured for each paper, the results being shown in the following table.

RELATIVE FLUORESCENT INTENSITY OF COLOR PHOTOGRAPHIC PRINTING PAPER AFTER COLOR PROCESSING

| Fluorescent brightening agent | High molecular weight compound |          |          |          | Polyvinyl pyrrolidone |
|-------------------------------|--------------------------------|----------|----------|----------|-----------------------|
|                               | None                           | Compd. 1 | Compd. 2 | Compd. 3 |                       |
| Leucophor B                   | 26                             | 72       | 69       | 72       | 57                    |
| Blankophor BUP                | 25                             | 71       | 68       | 71       | 55                    |
| Whitex BF                     | 25                             | 71       | 68       | 71       | 55                    |
| Kayaphor S                    | 24                             | 70       | 67       | 70       | 53                    |
| Tinopal GS                    | 24                             | 70       | 67       | 69       | 53                    |
| Compound 5                    | 21                             | 68       | 67       | 68       | 49                    |
| Compound 6                    | 22                             | 68       | 67       | 68       | 51                    |
| Compound 7                    | 60                             | 77       | 77       | 77       | 65                    |

As is clear from the above results, by using a combination of a known fluorescent brightening agent and the partially urethanated polyvinyl alcohol of this invention, very excellent brightening effects could be obtained. Also, the surface of the comparison printing paper containing polyvinyl pyrrolidone was matted and the image became opaque, while the printing paper containing the fluorescent brightening agent and the partially urethanated polyvinyl alcohol showed no such phenomenon.

10 1 g. of "Blankophor BUP" (trade name) and 10 g. of Compound 3 of this invention were added to 1 liter of a baryta-solution having the following composition, and the mixture was coated on a raw paper at the rate of 100 g./m.<sup>2</sup>.

|                | Baryta-solution |
|----------------|-----------------|
| Barium sulfate | 500 g.          |
| Gelatin        | 50 g.           |
| Chromium alum  | 2 g.            |
| Formalin (30%) | 0.3 ml.         |
| Water to make  | 1 liter         |

15 Onto the baryta-coated paper thus prepared was coated a composition prepared by adding a hardening agent and a wetting agent to a gelatino silver halide emulsion containing gelatin and pure silver chloride in a ratio of 10:4.

20 When the printing paper thus prepared was processed as in Example 1, the whiteness of the printing paper containing

40 Compound 3 in the baryta layer was not reduced by washing and the surface whiteness of the printing paper was better than the printing paper not containing the compound of this invention.

45 The same results were obtained when Compound 1, Compound 2, or Compound 4 was used instead of Compound 3 in this example.

## EXAMPLE 4

50 A coating composition prepared by adding 0.5 g. of "Tinopal GS" (trade name) as a fluorescent brightening agent and 12 g. of Compound 4 to 1 liter of a 5 percent aqueous gelatin solution containing 0.1 g. of colloidal nickel sulfide

70 was coated on a baryta-coated paper. To the layer thus prepared was applied a stripping layer consisting essentially of sodium alginate to give an image-receiving material for a diffusion transfer photographic process. The image-receiving material was brought into intimate contact with a light-sensitive material having a preliminary exposed silver halide emulsion layer image, and after immersing them in a developer, they were separated from each other after 30 minutes.

75 The whiteness of the highlight area of the positive image in

the case of using Compound 4 and the fluorescent brightening agent according to the present invention was better than when no compound of this invention was employed. Also, the same results were obtained when Compound 1, Compound 2, or Compound 3 was used instead of Compound 4 in this example.

The amount of the fluorescent brightening agent to be added to the layer may vary from 1 to 20 mg. per 100 cm.<sup>2</sup> of the layer.

What is claimed is:

1. A photographic printing paper comprising a paper support having thereon a light-sensitive silver halide emulsion layer containing a water-soluble fluorescent brightening agent and a partially urethanated polyvinyl alcohol having the following recurring structure:



wherein  $x+y$  is a number from 100 to 5,000 and  $y/(x+y)$  is a number from 0.05 to 0.25.

2. A photographic printing paper comprising a paper support having therein a light-sensitive silver halide emulsion layer and a subsidiary layer, at least one of said layers containing a water-soluble fluorescent brightening agent and a partially urethanated polyvinyl alcohol having the following recurring structure:



wherein  $x+y$  is a number from 100 to 5,000 and  $y/(x+y)$  is a number from 0.05 to 0.25.

3. The photographic printing paper as in claim 2 wherein said water-soluble fluorescent brightening agent and said partially urethanated polyvinyl alcohol are incorporated in said subsidiary layer which is a protective layer.

4. The photographic printing paper as in claim 2 wherein said water-soluble fluorescent brightening agent and said partially urethanated polyvinyl alcohol are incorporated in a light-sensitive silver halide emulsion layer.

5. The photographic printing paper as in claim 2 wherein said water-soluble fluorescent brightening agent and said par-

tially urethanated polyvinyl alcohol are incorporated in said subsidiary layer which is a baryta layer.

6. A photographic printing paper comprising a paper support having thereon a light-sensitive silver halide emulsion layer and a subsidiary layer, at least one of said layers containing a water-soluble fluorescent brightening agent and a partially urethanated polyvinyl alcohol having the following recurring structure:



wherein  $x+y$  is a number from 1,500 to 3,000 and  $y/(x+y)$  is a number from 7 to 20.

15 7. The photographic printing paper as in claim 6 wherein said water-soluble fluorescent brightening agent is a member selected from the group consisting of diaminostilbenes, benzidines, triazoles, imidazoles and imidazolones.

8. The photographic printing paper as in claim 6 wherein 20 said partially urethanated polyvinyl alcohol is 14 percent urethanated polyvinyl alcohol having a degree of polymerization of 2,400.

9. The photographic printing paper as in claim 6 wherein 25 said partially urethanated polyvinyl alcohol is 15 percent urethanated polyvinyl alcohol having a degree of polymerization of 1,700.

10. The photographic printing paper as in claim 6 wherein 30 said partially urethanated polyvinyl alcohol is 13 percent urethanated polyvinyl alcohol having a degree of polymerization of 2,400.

11. The photographic printing paper as in claim 6 wherein 35 said partially urethanated polyvinyl alcohol is 7 percent urethanated polyvinyl alcohol having a degree of polymerization of 2,400.

12. The photographic printing paper as in claim 6, wherein 40 said layer further contains a binder, and wherein the amount of said partially urethanated polyvinyl alcohol in said layer varies from 1 to 30 percent, by weight, based on the weight of the binder in said layer.

13. The photographic printing paper as in claim 1, wherein 45 said layer further contains a binder, and wherein the amount of said partially urethanated polyvinyl alcohol in said layer varies from 1 to 30 percent, by weight, based on the weight of the binder in said layer.

14. The photographic printing paper as in claim 2, wherein 50 said layer further contains a binder, and wherein the amount of said partially urethanated polyvinyl alcohol in said layer varies from 1 to 30 percent, by weight, based on the weight of the binder in said layer.

\* \* \* \* \*